

## UNITED STATES PATENT OFFICE

2,494,336

SEALING COMPOSITIONS AND PROCESSES  
FOR MAKING SAMEBernard Gross, San Diego, Calif., assignor to Rohr  
Aircraft Corporation, Chula Vista, Calif., a cor-  
poration of CaliforniaNo Drawing. Application July 28, 1945,  
Serial No. 607,675

6 Claims. (Cl. 260—29.2)

1

My invention relates to sealing compositions and processes for making same, and its objects are to produce a sealant which, when applied to cover joints of metallic parts, or openings therethrough or weaknesses therein, is impervious to oil or gasoline and at the same time is resistant to a considerable degree to open flame; to furnish a sealing composition which may not only be used as a sealant for such coverage, but also as a gasketing sealant under pressure of rivets or bolts; to bring about good adhesion of such sealant without the use of a special primer when applied directly to metal surfaces; to produce a composition which is rubber-like in character and capable of sustained vibrations without cracking or impairment of structure; to dispense with noxious odors and the use of inflammable material, and in general to furnish a more efficient flame, oil and gasoline resistant sealant than has heretofore been produced.

At the present time there are many types of sealing compositions on the market for sealing cracks or small openings occurring in or between metallic parts. These compositions are applied in the form of a liquid, a paste, or a putty; and after application either retain their original consistency, or change into a mass of different characteristics because of evaporation of solvents, or because of chemical changes brought about by heat, or because of reactions of chemicals combined therewith. None of these sealants, however, so far as I am aware, were capable of resisting both the deleterious action of oil or gasoline and even temporarily the effect of an open flame.

My improved sealant has, therefore, been brought into being to meet the need and demand for a sealing composition of these resistant characteristics. Such a sealant, for example, could be used on metal diaphragms behind an airplane engine to seal openings in sheet metal joints or at sheet metal corner relief holes. Also in the case of an airplane, through the use of my invention, the effect of fire upon such seal would ordinarily be avoided. In the absence of an effective flame sealant, should a fire break out of the engine of an airplane, and should a blast of air from the propeller thereof blow the flame against the metal of its aforesaid diaphragms (then acting as a fire wall), any melting of the

2

metal of the diaphragms would tend to start at the joints or relief holes and quickly spread therefrom. This would be because of the blast effect of the flame upon the edge of the metal at the joints or relief holes if the flame were allowed to pass therethrough. The rapid melting, which occurs after an initial start, results because the flame assisted by the blast of air always acts primarily upon the edge of the metal. However, if my flame resistant sealing compound were used to cover such joints or relief holes, the said flame would not contact the same and would be permitted to pass over the surface of the metal without detrimental consequences.

My sealing composition consists of a mixture of carbon black, zinc chromate, asbestos fibre and polyethylene formal polysulfide in which ingredients are mixed with water, preferably shortly prior to the application of the composition, and are applied in a paste form to cleaned metal parts without the necessity of a primer. These ingredients are mixed with a quantity of water sufficient to form a paste or mortar of such consistency as to enable it to be plastered over the surface of the parts to be sealed. It may be applied in one or more coats or layers in the ordinary manner according to the nature of the case and the degree of sealing required.

In preparing the said composition I prefer to combine the said ingredients in approximately the following proportions, viz.:

|                                                                                                                                 | Parts by weight |
|---------------------------------------------------------------------------------------------------------------------------------|-----------------|
| Polyethylene formal polysulfide dispersed in water 65 to 75% by weight                                                          | 159             |
| Carbon black, dispersed in water 40 to 50% by weight                                                                            | 8               |
| Zinc chromate, dispersed in water 30 to 40% by weight                                                                           | 4               |
| Asbestos fibre                                                                                                                  | 17 to 43        |
| Additional water (preferably 80 parts by weight may be added to prevent spoilage if the material is to be stored prior to use). |                 |

Preferably the zinc chromate and carbon black dispersion are mixed and kept in a container separate from a receptacle containing a mixture of the polyethylene formal polysulfide dispersion and asbestos; and the two are not combined until just prior to being plastered over the surface to be sealed. Soon after application of the

coat or layer of my improved sealant, such sealant so applied assumes a rubber-like consistency. If the sealant is to serve as a gasket between mating metal surfaces, it is spread in paste form over one of the mating surfaces, and after it acquires a rubber-like consistency with a shore hardness of approximately 50 to 60, it may be bolted or riveted to such mating metallic surface. If such mating surfaces are irregular, the sealant will cold flow and conform to the space between the mating metal surfaces. After this initial cold flow has taken place, the pressure of the bolts will cause the sealant to further cold cure to a shore hardness of between 60 to 70. After this has taken place, the gasket will not cold flow further under normal pressures produced by rivets or bolts for a given condition of mating surfaces.

My improved sealing composition is now being used successfully upon a production basis. Among other recognized advantages, are its excellent sealing properties against gasoline, oil and other petroleum products; its provision of good adhesion when applied directly to metal surfaces without the necessity of using a primer; its flame resistant qualities hereinbefore referred to; its rubber-like consistency and property of adhering without cracking to the surfaces to which it is applied notwithstanding the vibration thereof; its ability to permit without injury the use of cleaning fluids or other solvents; its use as a gasket under the conditions above set forth; and its freedom from obnoxious odors and inflammable ingredients.

If desired, particularly where protection from open flame is not desired or required, the ingredient of asbestos fibre could be dispensed with in the combinations of ingredients above referred to, and excellent results obtained from the use of a sealant made by a mixture of the remaining ingredients.

By the word "approximately" as used in the claims, I desire to be understood as using the word in its precise dictionary sense of approaching closely to the proportions recited without requiring exact coincidence therewith or substantial deviation therefrom.

My invention may be embodied in other specific forms without departing from the spirit or essential characteristics thereof. The present embodiment, as above set forth, is therefore to be considered in all respects as illustrative and not restrictive, the scope of my invention being indicated by the appended claims rather than by the above description, and all changes which come within the meaning and range of equivalency of the claims are therefore intended to be embraced therein.

What I claim and desire to secure by Letters Patent is:

1. A flame, oil and gasoline resistant sealing composition comprising approximately and by weight of (1) 159 parts of a water dispersion of polyethylene formal polysulfide, which is made up by weight of 65 to 75 percent polyethylene formal polysulfide and the balance water; (2) 8 parts of a water dispersion of carbon black, which is made up by weight of 40 to 50 percent carbon black and the balance water; (3) 4 parts of a water dispersion of zinc chromate which is made up by weight of 30 to 40 percent zinc chromate and the balance water; (4) 17 to 43 parts by weight of asbestos fibre.

2. A flame, oil and gasoline resistant sealing composition comprising approximately and by weight of (1) 159 parts of a water dispersion of polyethylene formal polysulfide, which is made up by weight of 65 to 75 percent polyethylene formal polysulfide and the balance water; (2) 8 parts of a water dispersion of carbon black, which is made up by weight of 40 to 50 percent carbon black and the balance water; (3) 4 parts of a water dispersion of zinc chromate which is made up by weight of 30 to 40 percent zinc chromate and the balance water; (4) 17 to 43 parts by weight of asbestos fibre; and (5) 80 parts of additional water.

3. A process for preparing a composition for sealing cracks and openings in metallic structures and applying the same comprising (1) mixing approximately and by weight (a) 159 parts of water dispersion of polyethylene formal polysulfide which is made up by weight of 65 to 75 percent polyethylene formal polysulfide and the balance water; (b) 8 parts of a water dispersion of carbon black which is made up by weight of 40 to 50 percent carbon black and the balance water; (c) 4 parts of a water dispersion of zinc chromate which is made up by weight of 30 to 40 percent zinc chromate and the balance water; and (5) 80 parts of additional water.

4. A process for preparing a composition for sealing cracks and openings in metallic structures and applying the same comprising (1) mixing approximately and by weight (a) 159 parts of water dispersion of polyethylene formal polysulfide which is made up by weight of 65 to 75 percent polyethylene formal polysulfide and the balance water; (b) 8 parts of a water dispersion of carbon black which is made up by weight of 40 to 50 percent carbon black and the balance water; (c) 4 parts of a water dispersion of zinc chromate which is made up by weight of 30 to 40 percent zinc chromate and the balance water; and (2) applying the mixture so formed to the area to be sealed.

5. A process for preparing a composition for sealing cracks and openings in metallic structures and applying the same comprising (1) mixing approximately and by weight (a) 159 parts of a water dispersion of polyethylene formal polysulfide which is made up by weight of 65 to 75 percent polyethylene formal polysulfide and the balance water; (b) 8 parts of a water dispersion of carbon black which is made up by weight of 40 to 50 percent carbon black and the balance water; (c) 4 parts of a water dispersion of zinc chromate which is made up by weight of 30 to 40 percent zinc chromate and the balance water; and (2) applying the mixture so formed to the area to be sealed.

6. A process for preparing a composition for sealing cracks and openings in metallic structures and applying the same which comprises (1) mixing approximately and by weight (a) 4 parts of a water dispersion of zinc chromate which is made up by weight of 30 to 40 percent zinc chromate and the balance water with (b) 8 parts of a water dispersion of carbon black which is made up by weight of 40 to 50 percent carbon black and the balance water; and (2) combining the mixture so formed with approximately and by weight 159 parts of a water dispersion of polyethylene formal polysulfide which is made up by weight of 65 to 75 percent of polyethylene formal polysulfide and the balance water; and (3) applying the paste so formed to the area to be sealed.

7. A process for preparing a composition for sealing cracks and openings in metallic structures against the deleterious action of flame, oil and gasoline and applying the same which comprises (1) mixing approximately and by weight (a) 4 parts of a water dispersion of zinc chromate which is made up by weight of 30 to 40 percent zinc chromate and the balance water with (b) 8 parts of a water dispersion of carbon black which is made up by weight of 40 to 50 percent carbon black and the balance water; (2) mixing approximately and by weight (a) 159 parts of a water dispersion of polyethylene formal polysulfide and the balance water; and (3) applying the paste so formed to the area to be sealed.

fide which is made up by weight of 65 to 75 percent of polyethylene formal polysulfide and the balance water with (b) 17 to 43 parts of asbestos fibre; (3) combining the mixture (1) with the mixture (2) and (4) applying the paste so formed to the area to be sealed.

BERNARD GROSS.

REFERENCES CITED

The following references are of record in the file of this patent:

UNITED STATES PATENTS

| Number    | Name        | Date          |
|-----------|-------------|---------------|
| 2,140,672 | Gray et al. | Dec. 20, 1938 |
| 2,186,284 | Denman      | Jan. 9, 1940  |
| 2,195,380 | Patrick     | Mar. 26, 1940 |
| 2,206,643 | Patrick     | July 2, 1940  |
| 2,219,550 | Martin, Jr. | Oct. 29, 1940 |

OTHER REFERENCES

10 Barron, "Modern Synthetic Rubbers," D. Van Nostrand Co. Inc., N. Y., 1944, page 285.